

# UNITED STATES PATENT OFFICE.

FREDERICK M. BECKET, OF NIAGARA FALLS, NEW YORK, ASSIGNOR TO ELECTRO METALLURGICAL COMPANY, OF NEW YORK, N. Y., A CORPORATION OF WEST VIRGINIA.

## METHOD OF TREATING IRON OR STEEL.

940,665.

No Drawing.

Specification of Letters Patent. Patented Nov. 23, 1909.

Application filed November 7, 1908. Serial No. 461,509.

To all whom it may concern:

Be it known that I, FREDERICK M. BECKET, a subject of the King of Great Britain, residing at Niagara Falls, in the county of 5 Niagara and State of New York, have invented certain new and useful Improvements in Methods of Treating Iron or Steel, of which the following is a specification.

This invention is a method of treating iron 10 or steel to remove therefrom gaseous and other impurities which exert a deleterious effect upon the metal, and to modify the properties of the metal by incorporating therewith the elements titanium, silicon and 15 carbon.

According to the invention there is incorporated with the molten metal, usually at the time of casting, an alloy or mixture containing titanium, silicon and carbon, preferably in proportions substantially as hereinafter described. This alloy possesses definite advantages for such use as compared with metallic titanium, ferro-titanium, or titanium carbid, in which forms the metal 20 titanium has heretofore been available for use in the treatment of iron or steel.

When titanium ores or ores of titanium and iron are reduced by carbon in an electric furnace, sufficient carbon being employed to insure fair commercial efficiency of the 30 operation, there is formed a product containing a large proportion of carbon, such proportion amounting in the case of titanium carbid to approximately twenty per cent. by weight of the product. A compound of this character is extremely hard, difficultly fusible, and dissolves but slowly in molten metal. It is moreover objectionable by reason of its 35 high carbon content, inasmuch as the quantity of the titanium compound which may be added to a given weight of iron or steel is necessarily limited by the carbon content permissible in the resulting metal.

I have discovered that by associating silicon in substantial proportions with the titanium, and by effecting the reduction under proper conditions, the proportion of carbon may be greatly reduced and the product acquires new and valuable characteristics. The 45 silicon in this case acts to some extent as a carbon-excluding agent.

It is essential that the titanium should be present in the alloy in proportion to render it of value for technical purposes, say in 50 excess of five per cent., and the percentage of

silicon should be sufficient to exert a marked effect upon the carbon content, that is to say to reduce the carbon content to ten per cent. or less. It should be understood that the percentage of silicon required to effect this 60 result is not fixed and invariable, but bears a general proportion to the percentage of titanium present, for the reason that a given percentage of silicon exerts less effect in reducing the carbon content of an alloy high 65 in titanium than is the case with an alloy relatively low in titanium.

An example of the composition of an alloy made in accordance with the present process is given in the following analysis: 70

|          |       |
|----------|-------|
| Titanium | 33.70 |
| Iron     | 43.69 |
| Silicon  | 14.23 |
| Carbon   | 8.32  |
| Aluminum | .08   |
| Calcium  | Trace |

In case of alloys lower in titanium the percentage of silicon above noted would yield a product of lower carbon content; and in case of alloys still richer in titanium it will be necessary to increase very considerably the percentage of silicon in order to maintain the carbon content of the alloy 80 within desirable limits. In case still lower carbon contents are desired, these can be secured by suitably increasing the proportion of silicon in the alloy. By using a high-grade rutile, products may be obtained containing less iron than is indicated by the 85 above analysis.

Titanium alloys produced in accordance with my process present as compared with ferro-titanium the advantages of a lower melting point and a capacity for entering 90 more freely into solution in molten iron or steel; furthermore, by reason of their comparatively low carbon content they may be added, if desired, in relatively large proportions without unduly increasing the proportion of carbon in the resulting metal. Their appearance varies somewhat in accordance with the mode of their production, rate of cooling, etc.; in general they have a 95 metallic luster and a more or less distinct metallic luster and a more or less distinct 100 crystalline fracture; they are very fusible as compared with titanium carbid or metallic titanium, and much softer than these products. They are comparatively brittle and are readily crushed to such state of sub- 105 110

division as is desirable for insuring their complete solution in molten iron or steel.

The process may be carried out under varying conditions, the essential feature being the reduction in an electric furnace of an ore containing titanium, in presence of carbon and of sufficient silicon to exclude from the product carbon in excess of ten per cent. The following methods are satisfactory: (1), 10 by reducing by carbon in an electric furnace a charge containing oxids of titanium and silicon; (2), by reducing oxid of titanium by carbon in an electric furnace, ferro-silicon or silicon being incorporated with 15 the charge or added to the bath. The carbon is usually employed in substantially the proportion required to unite with the oxygen of the oxid or oxids of the charge. In any case the process is preferably rendered continuous by adding fresh portions of the charge and removing the products from time to time.

In the treatment of iron or steel, the alloy in a suitable state of subdivision is added 20 to or incorporated with the molten metal, preferably at the time of casting. The proportion of alloy added depends upon the grade or character of the molten metal as well as upon the nature of the product de-

sired, as is well understood by those skilled in the art. It is not practicable to state with certainty the complete function of each ingredient of the above described alloy. It may be assumed however that the titanium acts chiefly upon the occluded nitrogen, and 35 the silicon upon the hydrogen and dissolved oxids. The result of the addition of the combined elements is to greatly improve the character of the iron or steel by reason of the elimination of a substantial proportion 40 of its impurities and the presence in the finished metal of the excess of titanium, silicon and carbon employed; and to produce a homogeneous and uniform product.

I claim:

The method of treating iron and steel, which consists in incorporating with the molten metal an alloy containing more than five per cent. each of titanium and silicon and less than ten per cent. of carbon, said 50 alloy being relatively fusible as compared with metallic titanium and titanium carbid.

In testimony whereof, I affix my signature in presence of two witnesses.

FREDK. M. BECKET.

Witnesses:

J. N. DEINHARDT,  
D. BURGESS.